# EUROPEAN PATENT SPECIFICATION

(11) **EP 1 273 652 B1**
(45) Date of publication and mention of the grant of the patent: **29.11.2006**
(21) Application number: 02254662.6
(22) Date of filing: 03.07.2002
(51) Int. Cl.: C10L 1/22, C10L 10/00

(54) **Fuel additive and fuel compositon containing the same**
Kraftstoffzusatz und denselben enthaltende Kraftstoffzusammensetzung
Additif pour combustible et composition de combustible le contenant

(30) Priority: 06.07.2001 JP 2001206390
(43) Date of publication of application: 08.01.2003
(73) Proprietor: Chevron Texaco Japan Ltd., Tokyo, 101-0041 (JP)
(72) Inventor: Ohta Satoshi,, Shizukoka (JP); Sugimoto Jun, Shizuoka (JP); Watanabe Hiroshi, Shizuoka (JP)
(74) Representative: Nash, David Allan

(56) References cited:
- EP-A- 0 012 345
- WO-A-98/16599
- DE-A- 3 709 195
- GB-A- 1 112 754
- US-A- 4 398 919

## Description

The present invention relates to a fuel additive containing an alkylene-oxide-adducted hydrocarbyl amide. In particular, the present invention relates to the use of the fuel additive in a gasoline fuel for the purpose of improving the acceleration performance and the driving performance of gasoline-fueled automobile engine.

### BACKGROUND OF THE INVENTION

In order to increase engine output power and acceleration response of spark ignition engines in automobiles, various types of oxygen-containing additives for hydrocarbon-based fuel have been investigated. These hydrocarbon-based fuels include alcohol (e.g. methanol and ethanol), ether (e.g. methyl-t-butyl ether), and ketone (e.g. acetone). In addition, the use of additives, such as hydrazine or nitro compounds (for example nitromethane including nitropropane and nitroparaffin, or nitrobenzene) have been examined for automobile racing. However, the problem with using such additives is that they often have an adverse effect on the durability of the engine and its components.

It is also known that organometallic compounds (e.g. tetraethyl lead or similar lead alkyls:ferrocene, methyl cyclopentadienyl manganese tricarbonyl), as well as aromatic amine compounds (e.g. aniline, monomethyl aniline, or dimethyl aniline) can be used as anti-knocking agents. However, it has been confirmed that these compounds dramatically reduce the operating efficiency of three-way catalysts due to catalyst poisoning.

Japanese Patent Application Number (Kokai) 58-104996 (corresponding to US Patent Number 4,409,000) describes the use of an alkyl amine or ethyleneoxide-adducted alkenyl amine as an additive in automobile fuel to clean carburetors and engines.

WO 98/16599 discloses monoamide-containing polyether alcohol compounds of formula R1-C(O)-N(R₂,R₃), wherein R₁, R₂, and R₃ are each independently selected from hydrogen, hydrocarbyl of 1 to 100 carbon atoms, susbtituted hydrocarbyl of 1 to 100 carbon atoms and polyoxyalkylene alcohol of 2 to 200 carbon atoms or R₂ and R₃ taken together form a heterocyclic group of 2 to 100 carbon atoms or a substituted heterocyclic group of 2 to 100 carbon atoms with the proviso that at least one of R₁, R₂ or R₃ must be polyoxyalkylene alcohol. These compounds have been found to decrease intake valve deposits, control octane requirement increases and reduce octane requirement when used as gasoline additives.

EP 0012345 discloses a fuel for an automobile, internal combustion engine or a diesel engine comprising a hydrocarbon, water and emulsifier wherein the emulsifier is a non-ionic emulsifier and comprises the addition product of ethylene oxide or propylene oxide and a carboxylic acid amide with 9 to 21 carbon atoms.

In DE 3709195 storage-stable emulsifier formulations are proposed which comprise non-ionic emulsifiers, water, and possibly solvents, which contain 50-95% non-ionic emulsifiers or emulsifier mixtures, preferably degradable emulsifiers, 3-30%, preferably 3-20% water and possibly 0-30% solubiliser, such as C₁-C₁₀ straight-chain and branched-chain alcohols, C₁₀-C₁₈ unsaturated alcohols, aromatic compounds, preferably toluene and xylene, aliphatic compounds, preferably C₇-C₂₀ hydrocarbons, which can be branched or cyclic. Non-ionic emulsifiers of the formula R-C(O)-N(Yₙ,R₁) are preferably used for this, in which R denotes an un-substituted or substituted radical which can be a straight-chain or branched or cyclic, saturated or unsaturated hydrocarbon radical, Y represents the group -CH₂-CH₂(R₂)-O- in which R₂ is H or methyl, n is a number from 1-50, preferably a mixture of 1-3 and 5-20, and R₁ represents H or the group Yₙ-H and which possibly contain monoglycerides of the corresponding fatty acids as a result of the production method.

US 4,398,919 is directed to aqueous-comminuted coal slurries. Specifically, it is directed to slurries that include as surfactants about 0.1 to 0.5 weight percent surfactant compounds, as for example polyoxyethylene (2) oleamide, and which typically have a coal solids content of 70%.

According to European Patent Number 0869163 A1 it is possible to reduce friction in gasoline engines by adding N,N-bis(hydroxyalkyl) alkyl amine to gasoline.

According to PCT Patent Publication 2001-502374 (WO-98/17745), solubility in water as well as the engine performance can be improved by adding fatty acid diethanol amide, fatty acid ethoxylate and alcohol ethoxylate to a liquid fuel such as gasoline or diesel fuel.

### SUMMARY OF THE INVENTION

In its broadest aspect, the present invention relates to the use of a fuel additive comprising an alkylene-oxide-adducted hydrocarbyl amide having from 3 to 50 moles of alkylene oxide per mole of hydrocarbyl amide in a gasoline fuel for the purpose of improving the acceleration performance of a gasoline fueled automobile engine. The fuel additive may be present in an amount, from 10 to 10,000 ppm weight per weight of fuel.

Among other factors, the present invention is based on the discovery that certain alkylene-oxide-adducted hydrocarbyl amides are surprisingly useful for improving the acceleration response and the driving performance of internal combustion engines when used as fuel additives in gasoline fuels.

### DETAILED DESCRIPTION OF THE INVENTION

As stated above, the present invention relates to the use of a fuel additive containing an alkylene-oxide-adducted hydrocarbyl amide in a gasoline fuel.

Prior to discussing the present invention in detail, the following terms will have the following meanings unless expressly stated to the contrary.

### Definitions

The term "hydrocarbyl" refers to an organic radical primarily composed of carbon and hydrogen which may be aliphatic, alicyclic, aromatic or combinations thereof, e.g., aralkyl or alkaryl. Such hydrocarbyl groups may also contain aliphatic unsaturation, i.e., olefinic or acetylenic unsaturation, and may contain minor amounts of heteroatoms, such as oxygen or nitrogen, or halogens, such as chlorine. When used in conjunction with carboxylic fatty acids, hydrocarbyl will also include olefinic unsaturation.

The term "alkyl" refers to both straight- and branched-chain alkyl groups.

The term "lower alkyl" refers to alkyl groups having 1 to about 6 carbon atoms and includes primary, secondary and tertiary alkyl groups. Typical lower alkyl groups include, for example, methyl, ethyl, n-propyl, isopropyl, n-butyl, sec-butyl, t-butyl, n-pentyl, n-hexyl and the like.

The term "alkenyl" refers to an alkyl group with unsaturation.

The term "alkylene oxide" refers to a compound having the formula: wherein R₁ and R₂ are each independently hydrogen or lower alkyl having from 1 to 6 carbon atoms.

The term "fuel" or "hydrocarbon-based fuel" refers to normally liquid hydrocarbons having boiling points in the range of gasoline and diesel fuels.

In its broadest aspect, the present invention involves the use of a fuel additive comprising an alkylene-oxide-adducted hydrocarbyl amide having from 3 to 50 moles, preferably from 3 to 20 moles, more preferably from 4 to 15 moles, of alkylene oxide per mole of hydrocarbyl amide in a gasoline fuel for the purpose of improving the acceleration performance of a gasoline-fueled automobile engine.

The alkylene-oxide-adducted hydrocarbyl amide used in the present invention is derived from an alkyl amide having from 4 to 75, preferably from 8 to 22, carbon atoms or alkenyl amide with at least one or two points of unsaturation having from 4 to 75, preferably from 8 to 22, carbon atoms. Examples of desirable alkyl amides suitable for the present invention include, but are not limited to, octyl amide (capryl amide), nonyl amide, decyl amide (caprin amide), undecyl amide dodecyl amide (lauryl amide), tridecyl amide, teradecyl amide (myristyl amide), pentadecyl amide, hexadecyl amide (palmityl amide), heptadecyl amide, octadecyl amide (stearyl amide), nonadecyl amide, eicosyl amide (alkyl amide), or docosyl amide (behenyl amide). Examples of desirable alkenyl amides include, but are not limited to, palmitoolein amide, oleyl amide, isooleyl amide, elaidyl amide, linolyl amide, linoleyl amide. Preferably, the alkyl or alkenyl amide is a coconut oil fatty acid amide.

The alkylene oxide adducted to the hydrocarbyl amide used in the present invention is derived from an alkylene group having from 2 to 5 carbon atoms. Preferably, the alkylene oxide is selected from the group consisting of ethylene oxide, propylene oxide, butylene oxide, and pentylene oxide. Ethylene oxide and propylene oxide are particularly preferred. In addition, mixtures of alkylene oxides are desirable in which, for example, a mixture of ethylene oxide and propylene oxide may be used to form the alkylene-oxide-adducted hydrocarbyl amide of the present invention. A respective molar ratio of from 1:5 to 5:1 may be used in the case of a mixture of ethylene oxide and propylene oxide.

A desirable number of moles of the alkylene oxide to be adducted to the hydrocarbyl amide will be in the range of from 3 to 50 moles of alkylene oxide per 1 mole of hydrocarbyl amide. More preferably, the range of from 3 to 20 moles is particularly desirable. Most preferably, the range of from 4 to 15 moles is most preferable as a molar range of the additive.

Preferably, the alkylene-oxide adducted hydrocarbon amide is derived from an alkylene-oxide-adduction reaction involving a coconut oil fatty acid amide with ethylene oxide and propylene oxide. However, the alkylene-oxide adducted hydrocarbyl amides useful as fuel additives in the present invention can be also a mixed product wherein various types and different moles of alkylene oxide and can be adducted to various types of hydrocarbyl amides.

The amount of fuel additive present in a gasoline fuel will typically be in a range of from 10 to 10,000 ppm weight per weight (active component ratio). More preferably, the desired range is from 10 to 5,000 ppm weight per weight, while a range of from 10 to 1,000 ppm weight per weight is most preferable.

The fuel additive of the present invention is normally supplied as an organic solvent solution with an effective fuel additive content of at least 30 weight %, based on the amount of the fuel additive and organic solvent solution.

Although no particular limitations are imposed on the method used to add a fuel additive of the present invention to a hydrocarbon-based fuel, a concentrated fuel additive product may be prepared which contained at least 30 weight % of the active component. This product can be added according to any selected method including adding it into the fuel tank of a fuel station or into the fuel tank of a passenger car.

The fuel additive used in the present invention can also be combined with one, two, or more other additives publicly known to be used in hydrocarbon-based fuels. Such additives include, but are not limited to, deposit control additives such as detergents or dispersants, corrosion inhibitors, oxidation inhibitors, metal deactivators, corrosion inhibitors, demulsifiers, static electricity preventing agents, anti-coagulation agents, anti-knock agents, oxygenates, flow improvers, pour point depressants, cetane improvers and auxiliary-solution agents.

### EXAMPLES

The invention will be further illustrated by the following examples, which set forth particularly advantageous method embodiments. While the examples are provided to illustrate the present invention, they are not intended to limit it. The present invention has been described with reference to specific embodiments and it is intended to cover those various changes and substitutions that may be made by those skilled in the art without departing from the spirit and scope of the appended claims.

### Example 1

A Toyota Camry 1800cc, 5MT (Type E-SV40, provided with Knock Sensor, type 4S-FE engine), mounted on a chassis dynamometer, was operated at a constant speed of 20 km/hr. The acceleration measurement was initiated by fully opening the throttle and measuring the amount of time required for the vehicle speed to reach 110 km/hr with the transmission locked in fourth gear. This measurement was repeated 10 times using the same fuel and the median value obtained from these 10 measurements was determined as the acceleration time period. In addition, in order to minimize the influence of ambient conditions (temperature, pressure, etc.) on engine performance, the entire test procedure was executed within a single day.

The gasoline used have the following specifications: density (at 15°C): 0.7389 g/cm³, Reid vapor pressure: 60.5 Kpa, octane number: 90.2 (RON), 82.3 (MON), aromatics (volume %): 29.9, olefin (volume %): 15.6, 10% distillation temperature (°C): 50.0, 50% distillation temperature (°C): 92.0, 90% distillation temperature (°C): 169.5. The fuel composition was adjusted by adding 100mg/L of 5 moles of oleyl amide-ethylene oxide (fuel additive) to this gasoline.

Gasoline containing the above described fuel additive and gasoline without the fuel additive (same as the above) were then tested in accordance with the test procedures described herein above. Table 1 shows the results.

**Table 1**

| Test Fuel Oil | Acceleration Time Period (20 -110km/hours) |
|---|---|
| Gasoline with No Additive | 24.91 seconds |
| (Comparative Example) | |
| Fuel Composition containing Additive | 24.69 seconds |

From the different acceleration time periods shown in Table 1, it is clear that the acceleration performance was improved by the fuel additive of the present invention. Although the difference in the acceleration time period indicated in Table 1 is not dramatic (less than 1%) with the fuel additive of the present invention, this is a distinct difference, particularly in case of cars needing to attain a high speed, such as racing cars, etc. Furthermore, in addition to the importance of acceleration for racing cars, even a small improvement in acceleration performance can be very important for passenger cars driving on public roads where it may be necessary to suddenly accelerate in order to avoid an accident, etc., as a result of a sudden event.

### Example 2

The test was carried out as described in Example 1, using four moles of propylene oxide adducted coconut oil fatty acid di-ethanol amide (fuel additive) was added at a concentration of 100 mg/L to this gasoline in order to prepare a fuel composition containing the fuel additive.

Gasoline containing the above described fuel additive and gasoline without the fuel additive (same as the above) were then tested in the acceleration evaluation test in accordance with the test procedures described in Example 1. Table 2 shows the results of the test.

**Table 2**

| Test Fuel Oil | Acceleration Time Period (20 -110km/hours) |
|---|---|
| Gasoline with No Additive | 24.51 seconds |
| (Comparative Example) | |
| Fuel Composition containing Additive | 24.38 seconds |

As shown by the results in Table 2, the acceleration performance was clearly improved when the fuel additive of the present invention was employed in the fuel.

### Example 3

The test was carried out as described in Example 1, using ten moles of propylene oxide adducted coconut oil fatty acid di-ethanol amide (fuel additive) was added to provide a concentration of 100 mg/L in this gasoline in order to prepare a fuel composition containing the fuel additive.

Gasoline containing the above described fuel additive and gasoline without fuel additive (same as the above) were then tested in accordance with the test procedures described previously. Table 3 shows the results of the test.

**Table 3**

| Test Fuel Oil | Acceleration Time Period (20 -110km/hours) |
|---|---|
| Gasoline with No Additive | 24.85 seconds |
| (Comparative Example) | |
| Fuel Composition containing Additive | 24.74 seconds |

As shown by the results in Table 3, the acceleration performance was clearly improved when the fuel additive of the present invention was employed in the fuel.

### Example 4

The test was carried out as described in Example 1 except the gasoline used had the following specifications: density 9 at 15°C: 0.7303 g/cm³, Reid vapor pressure: 60.2Kpa, octane number: 92.1 (RON), aromatics (volume %): 23.19, olefin (volume %) 19, 10% distillation temperature (°C): 54.3, 50% distillation temperature (°C): 86.2, 90% distillation temperature (°C): 158.1 and using four moles of propylene oxide and two moles of ethylene oxide adducted coconut oil fatty acid di-ethanol amide (fuel additive) were added to provide a concentration of 100 mg/L in this gasoline.

Gasoline containing the above described fuel additive and gasoline without fuel additive (same as the above) were then tested in accordance with the test procedures described previously. Table 4 shows the results of the test.

**Table 4.**

| Test Fuel Oil | Acceleration Time Period (20 -110km/hours) |
|---|---|
| Gasoline with No Additive | 23.96 seconds |
| (Comparative Example) | |
| Fuel Composition containing Additive | 23.75 seconds |

As shown by the results in Table 4, the acceleration performance was clearly improved when the fuel additive of the present invention was employed in the fuel.

## Claims

1. The use of a fuel additive comprising an alkylene-oxide-adducted hydrocarbyl amide having from 3 to 50 moles of alkylene oxide per mole of hydrocarbyl amide in a gasoline fuel for the purpose of improving the acceleration performance of a gasoline-fueled automobile engine.

2. The use of a fuel additive according to Claim 1, wherein the alkylene-oxide-adducted hydrocarbyl amide has from 3 to 20 moles of alkylene oxide per mole of hydrocarbyl amide.

3. The use of a fuel additive according to Claim 2, wherein the alkylene-oxide-adducted hydrocarbyl amide has from 4 to 15 moles of alkylene oxide per mole of hydrocarbyl amide.

4. The use of a fuel additive according to Claim 1, wherein the alkylene-oxide-adducted hydrocarbyl amide is derived from an alkyl or alkenyl amide having from 4 to 75 carbon atoms.

5. The use fo a fuel additive according to Claim 4, wherein the alkylene-oxide-adducted hydrocarbyl amide is derived from an alkyl or alkenyl amide having from 8 to 22 carbon atoms.

6. The use of a fuel additive according to Claim 5, wherein the alkyl or alkenyl amide is a coconut oil fatty acid amide.

7. The use of a fuel additive according to Claim 1, wherein the alkylene oxide is selected from the group consisting of ethylene oxide, propylene oxide, butylene oxide, pentylene oxide, or mixtures thereof.

8. The use of a fuel additive according to Claim 7, wherein the alkylene oxide is elected from the group consisting of ethylene oxide, propylene oxide, or a mixture thereof.

9. The use of a fuel additive according to Claim 1, wherein the alkylene-oxide-adducted hydrocarbyl amide is derived from an alkylene-oxide-adduction reaction involving a coconut oil fatty acid amide with ethylene oxide and propylene oxide.

10. The use of a fuel additive according to claim 1, wherein the amount of alkylene oxide is from 3 to 20 moles per mole of hydrocarbyl amide and said alkylene oxide is selected from the group consisting of ethylene oxide, propylene oxide, butylene oxide, pentylene oxide, or mixtures thereof.

11. The use as claimed in any proceeding claim, wherein the fuel additive is present in an amount of from 10 to 10,000 ppm weight per weight of fuel.

12. The use according to Claim 11, wherein the alkylene-oxide-adducted hydrocarbyl amide is in the range of from 10 to 5,000 ppm weight per weight of fuel.

13. The use according to Claim 12, wherein the alkylene-oxide-adducted hydrocarbyl amide is in the range of from 10 to 1000 ppm weight per weight of fuel.

## Patentansprüche

1. Verwendung eines Kraftstoffadditivs, umfassend ein Kohlenwasserstoffamid-Alkylenoxid-Addukt mit 3 bis 50 Mol Alkylenoxid pro Mol Kohlenwasserstoffamid in einer Benzinbeschickung zum Verbessern der Beschleunigungsleistung eines benzinbetriebenen Automotors.

2. Verwendung eines Kraftstoffadditivs nach Anspruch 1, wobei das Kohlenwasserstoffamid-Alkylenoxid-Addukt 3 bis 20 Mol Alkylenoxid pro Mol Kohlenwasserstoffamid aufweist.

3. Verwendung eines Kraftstoffadditivs nach Anspruch 2, wobei das Kohlenwasserstoffamid-Alkylenoxid-Addukt 4 bis 15 Mol Alkylenoxid pro Mol Kohlenwasserstoffamid aufweist.

4. Verwendung eines Kraftstoffadditivs nach Anspruch 1, wobei das Kohlenwasserstoffamid-Alkylenoxid-Addukt hergeleitet ist von einem Alkyl- oder Alkenylamid mit 4 bis 75 Kohlenstoffatomen.

5. Verwendung eines Kraftstoffadditivs nach Anspruch 4, wobei das Kohlenwasserstoffamid-Alkylenoxid-Addukt hergeleitet ist von einem Alkyl- oder Alkenylamid mit 8 bis 22 Kohlenstoffatomen.

6. Verwendung eines Kraftstoffadditivs nach Anspruch 5, wobei das Alkyl- oder Alkenylamid ein Kokosölfettsäureamid ist.

7. Verwendung eines Kraftstoffadditivs nach Anspruch 1, wobei das Alkylenoxid ausgewählt ist aus der Gruppe Ethylenoxid, Propylenoxid, Butylenoxid, Pentylenoxid oder Gemischen davon.

8. Verwendung eines Kraftstoffadditivs nach Anspruch 7, wobei das Alkylenoxid ausgewählt ist aus der Gruppe Ethylenoxid, Propylenoxid oder einem Gemisch davon.

9. Verwendung eines Kraftstoffadditivs nach Anspruch 1, wobei das Kohlenwasserstoffamid-Alkylenoxid-Addukt hergeleitet ist von einer Alkylenoxid-Additionsreaktion, an der ein Kokosölfettsäureamid mit Ethylenoxid und Propylenoxid beteiligt ist.

10. Verwendung eines Kraftstoffadditivs nach Anspruch 1, wobei die Menge Alkylenoxid von 3 bis 20 Mol pro Mol Kohlenwasserstoffamid reicht und das Alkylenoxid ausgewählt ist aus der Gruppe Ethylenoxid und Propylenoxid, Butylenoxid, Pentylenoxid oder Gemischen davon.

11. Verwendung nach einem vorhergehenden Anspruch, wobei das Kraftstoffadditiv in einer Menge von 10 bis 10000 ppm Gewicht pro Kraftstoffgewicht zugegen ist.

12. Verwendung nach Anspruch 11, wobei das Kohlenwasserstoffamid-Alkylenoxid-Addukt im Bereich von 10 bis 5000 ppm Gewicht pro Kraftstoffgewicht ist.

13. Verwendung nach Anspruch 12, wobei das Kohlenwasserstoffamid-Alkylenoxid-Addukt im Bereich von 10 bis 1000 ppm Gewicht pro Kraftstoffgewicht ist.

## Revendications

1. Utilisation d'un additif pour carburants, comprenant un produit d'addition oxyde d'alkylène-hydrocarbylamide comprenant 3 à 50 moles d'oxyde d'alkylène par mole d'hydrocarbylamide, dans un moteur à essence afin d'améliorer les performances d'accélération d'un moteur d'automobile alimenté à l'essence.

2. Utilisation d'un additif pour carburants suivant la revendication 1, dans laquelle le produit d'addition oxyde d'alkylène-hydrocarbylamide comprend 3 à 20 moles d'oxyde d'alkylène par mole d'hydrocarbylamide.

3. Utilisation d'un additif pour carburants suivant la revendication 2, dans laquelle le produit d'addition oxyde d'alkylène-hydrocarbylamide comprend 4 à 15 moles d'oxyde d'alkylène par mole d'hydrocarbylamide.

4. Utilisation d'un additif pour carburants suivant la revendication 1, dans laquelle le produit d'addition oxyde d'alkylène-hydrocarbylamide est dérivé d'un alkyl- ou alcénylamide comprenant 4 à 75 atomes de carbone.

5. Utilisation d'un additif pour carburants suivant la revendication 4, dans laquelle le produit d'addition oxyde d'alkylène-hydrocarbylamide est dérivé d'un alkyl- ou alcénylamide comprenant 8 à 22 atomes de carbone.

6. Utilisation d'un additif pour carburants suivant la revendication 5, dans laquelle l'alkyl- ou l'alcénylamide est un amide d'acides gras d'huile de copra.

7. Utilisation d'un additif pour carburants suivant la revendication 1, dans laquelle l'oxyde d'alkylène est choisi dans le groupe consistant en oxyde d'éthylène, oxyde de propylène, oxyde de butylène, oxyde de pentylène et leurs mélanges.

8. Utilisation d'un additif pour carburants suivant la revendication 7, dans laquelle l'oxyde d'alkylène est choisi dans le groupe consistant en oxyde d'éthylène, oxyde de propylène et un de leurs mélanges.

9. Utilisation d'un additif pour carburants suivant la revendication 1, dans laquelle le produit d'addition oxyde d'alkylène-hydrocarbylamide provient d'une réaction d'addition d'oxyde d'alkylène impliquant un amide d'acides gras de l'huile de copra avec l'oxyde d'éthylène et l'oxyde de propylène.

10. Utilisation d'un additif pour carburants suivant la revendication 1, dans laquelle la quantité d'oxyde d'alkylène est de 3 à 20 moles par mole d'hydrocarbylamide et ledit oxyde d'alkylène est choisi dans le groupe consistant en oxyde d'éthylène, oxyde de propylène, oxyde de butylène, oxyde de pentylène et leurs mélanges.

11. Utilisation suivant l'une quelconque des revendications précédentes, dans laquelle l'additif pour carburants est présent en une quantité de 10 à 10 000 ppm en poids par poids de carburant.

12. Utilisation suivant la revendication 11, dans laquelle le produit d'addition oxyde d'alkylène-hydrocarbyl-amide est présent en une quantité comprise dans l'intervalle de 10 à 5000 ppm en poids par poids de carburant.

13. Utilisation suivant la revendication 12, dans laquelle le produit d'addition oxyde d'alkylène-hydrocarbyl-amide est présent en une quantité comprise dans l'intervalle de 10 à 1000 ppm en poids par poids de carburant.
